

## UNITED STATES PATENT OFFICE

1,959,509

## COPPER BASE ALLOY

Sam Tour, Englewood, N. J., assignor to Lucius  
Pitkin, Inc., a corporation of New YorkNo Drawing. Application June 14, 1930,  
Serial No. 461,260

7 Claims. (Cl. 75—1)

Many copper base alloys have been used for industrial purposes notwithstanding the difficulties which have been encountered in producing and working them. An important series of such 5 alloys has contained copper and silicon, either with or without the addition of other metals such as zinc, iron, manganese, nickel, cobalt, etc., in various proportions. Such alloys are advantageous because of their ductility and tenacity due 10 to the presence of copper, hardness imparted by the silicon, and other properties as contributed or modified by the other metals. One serious objection to these alloys, however, is that they are quite tough and stringy and therefore difficult 15 to machine,—so much so that their use has been somewhat limited.

It is desirable for many purposes to provide copper base alloys with free cutting qualities, and this has been done in the past by adding lead 20 to such alloys which do not contain silicon. Experience has shown that the addition of lead to copper alloys containing silicon does not give the desired machinability and free cutting properties, for the reason that the lead reacts with 25 the silicon to form a silicide which causes localized hard spots and decided amounts of segregation, etc., as well as causing loss of lead from the molten metal during the melting. It has therefore been necessary in the past to sacrifice 30 the properties imparted by the silicon in order to obtain increased machinability, but the present invention overcomes the above-mentioned and other objectionable features of the prior art 35 and provides a copper base alloy including silicon and a metal other than lead.

In solving this problem, I have found that bismuth, contrary to the accepted teachings of the art, is exceptionally well suited for increasing the machinability of copper-silicon alloys 40 without sacrificing any important properties. Thus, in carrying out the invention, I provide a copper base alloy with silicon containing from 1% to 6% of bismuth, this alloy giving excellent 45 results regardless of whether it is of the yellow brass variety (approximately 60% copper), or of the red brass or bronze variety (approximately 80% or more copper). Of course, the amount of bismuth to be added to any given copper base 50 alloy containing silicon is variable, dependent upon the basic properties of that alloy without the bismuth, and upon the degree of free cutting qualities desired. In fact, the invention is susceptible of numerous variations in the relative 55 proportions of the component elements.

By way of example, the new alloy may contain

50% or more of copper, .1% or more of silicon, and from 1% to 6% of bismuth. These three elements may be mixed together to constitute the only components of the alloy, or other metals may be added to them. Thus, modifications of 60 the invention may include iron, manganese, and/or zinc in the proportion of .1% or more of each or of any one of them, in addition to the copper, silicon, and bismuth. In referring to the percentages of silicon, iron, manganese and zinc 65 as being .1% or more, I have in mind the percentages used heretofore in producing alloys of these metals, it being known that the percentages above the minimum may vary to a considerable extent. My invention consists primarily in adding to these known alloys a percentage of bismuth sufficient to produce the desired results. Of course, my invention is not intended to be 70 confined to such known alloys and is believed to be applicable to any copper base alloy containing 75 silicon.

The new alloy embodying the invention can be readily produced by merely melting the constituent elements in any preferred type of furnace and stirring them together in a manner 80 well known to those skilled in the art. The bismuth in the mixture greatly increases the fluidity of the alloy in the molten state and this, coupled with the fact that the bismuth reduces the overall shrinkage in cooling, renders the alloy 85 particularly well adapted for casting purposes, giving much sharper detail than has been possible with prior art copper base alloys. However, the alloy is not limited to use as a casting metal, but, by reason of its ductility and malleability, 90 it can be worked either hot or cold by rolling, heating, spinning, drawing, or otherwise, as desired. And, as previously stated, it possesses to a high degree the much desired free cutting 95 properties which make possible its easy machining, whether by drilling, boring, turning, shaping, filing, or otherwise.

Having thus described my invention, what I claim is:

1. An alloy consisting of 1 to 6% bismuth, .1 to 6% silicon, .1 to 35% zinc and .1 to 6% of one or more metals of the group consisting of iron, manganese, nickel and cobalt, and the remainder substantially copper.
2. The method of rendering machinable, an alloy 105 consisting of copper or copper and one or more elements of the group consisting of zinc, iron, manganese, nickel and cobalt to which silicon has been added for the purpose of hardening, said method consisting in adding bismuth to the 110

alloy in quantities sufficient to produce the desired degree of machineability.

3. The method of imparting fluidity to an alloy in the molten state, consisting of copper or 5 copper and one or more elements of the group consisting of zinc, iron, manganese, nickel and cobalt, and to which silicon has been added for the purpose of hardening, said method consisting in adding bismuth to the alloy in quantities 10 sufficient to produce the desired degree of fluidity.
4. A copper base alloy containing from about .1 to 6% silicon, about 1 to 6% bismuth and characterized by being readily machineable due to the presence of bismuth.
- 15 5. A copper base alloy containing from about

.1 to 6% silicon, about 1 to 6% bismuth and characterized by having increased fluidity in its molten state due to the presence of bismuth.

6. A copper base alloy containing from about .1 to 6% silicon, about 1 to 6% bismuth, about 80 .1 to 35% zinc and characterized by being readily machineable due to the presence of bismuth.

7. A copper base alloy containing from about .1 to 6% silicon, about 1 to 6% bismuth, about .1 to 6% of one or more metals of the group, 85 consisting of iron, manganese, nickel and cobalt and characterized by being readily machineable due to the presence of bismuth.

SAM TOUR. 90

20 95

25 100

30 105

35 110

40 115

45 120

50 125

55 130

60 135

65 140